

Nov. 26, 1929.

M. KLEIFOTH

1,737,286

TAPERED FIBROUS SHEET

Filed Oct. 20, 1928

2 Sheets-Sheet 1



INVENTOR  
Max Kliefoth  
BY  
Pannie, Davis, Marrin & Edwards  
ATTORNEYS

Nov. 26, 1929.

M. KLIEOFTH

1,737,286

TAPERED FIBROUS SHEET

Filed Oct. 20, 1928

2 Sheets-Sheet 2

Fig. 6.



Fig. 7.



Fig. 8.



Fig. 9.



Fig. 11.



Fig. 10.



INVENTOR

Max Kliefotth

BY

Pennie, Davis, Marvin & Edmunds  
ATTORNEYS

## UNITED STATES PATENT OFFICE

MAX KLEFOTH, OF MADISON, WISCONSIN, ASSIGNOR TO C. F. BURGESS LABORATORIES, INC., OF MADISON, WISCONSIN, A CORPORATION OF DELAWARE

## TAPERED FIBROUS SHEET

Application filed October 20, 1928. Serial No. 313,687.

This invention relates to a fibrous material in the form of sheets of varying thickness such as tapered fibrous shingles and to a method of making such fibrous material.

5 This invention is an improvement over the process disclosed in the H. F. Weiss application Serial No. 139,476 filed October 4, 1926. One of the objects of my invention is to provide an improved continuous method for making a tapered fibrous shingle on a one cylinder machine. A further object of this invention is to make a continuous fibrous sheet of successively increasing and decreasing thickness along the machine direction of the 10 sheet. It is still a further object to provide a fibrous shingle in which the degree of taper may be varied at will.

Other objects, advantages and characteristic features will become apparent from the 20 following description of my new product and process and from the accompanying drawings wherein:

Fig. 1 is a diagrammatic plan view of the apparatus which is used to make one form 25 of my improved fibrous sheet;

Fig. 2 is a vertical, sectional view taken along line 2—2 of Fig. 1;

Fig. 3 is a portion of a sheet produced by the apparatus of Figs. 1 and 2;

30 Fig. 4 is a diagrammatic side view of another machine used to make another form of fibrous sheet;

Fig. 5 is a plan view of a sheet laid down in accordance with the modification shown in 35 Fig. 4;

Fig. 6 is an exaggerated longitudinal section through a fibrous sheet before pressing and as laid down in accordance with the modification of my improved method shown in 40 Fig. 4;

Fig. 7 is an exaggerated longitudinal section through my double tapered board after pressing;

Fig. 8 is a reproduction of Fig. 7 with the 45 contour of the board greatly exaggerated;

Fig. 9 is a greatly exaggerated longitudinal section through the board after it has undergone a final shaping and drying operation;

50 Fig. 10 is a side view of a shaping and drying press roll; and

Fig. 11 is a diagrammatic side view of a preliminary drier which may be included in the machines of Figs. 1, 2 and 4.

Although several methods are described in the Weiss application for the production of 55 tapered fibrous shingles, on the machine described therein, I have discovered a new and improved method for accomplishing the same result by a change in the apparatus used by Weiss, thereby changing the methods 60 described by him. By my improved method I form a continuous fibrous sheet of successively increasing and decreasing thickness along the machine direction of the sheet. This sheet is then cut at the lines of minimum 65 and maximum thickness to produce tapered shingles.

The composition of and the method of making my improved product can best be understood by referring to the accompanying drawings in which like numerals indicate like parts in the several figures. The vat 1 of a wet machine contains the slurry of water and pulp. The usual perforate cylinder mould 2 picks up a web of pulp which is then carried to couch roll 3, around which felt 4 travels in the indicated direction. The wet pulp web is picked up and carried along on felt 4 from the perforate cylinder mould 2 and is then pressed by press roll 5. The moist 70 pulp web is picked up by press roll 5 and is removed therefrom by doctor 6. This pulp web may be creped by the doctor or may be kept smooth as desired. In order to secure 75 a high degree of smoothness, the web may be arranged to be transferred from roll 5 to conveyor belt 7 without coming in contact with the doctor 6. The pulp web 8 is then carried forward by a conveyor belt 80 7 which is part of a hinged reciprocating looping device which is shown in another position by the dotted lines of Fig. 2. The off-take roll 9 of the hinged looping device works along a guide 10 and distributes the pulp web 8 across the conveyor 11 as shown.

Tightener roll 12 functions to keep conveyor belt 7 taut and directs the return travel of belt 7 along a path which is at all times as nearly as possible of the same length as the forward path. In Figs. 1 and 2 the pulp web 85 90 95 100

is distributed transversely on the conveyor 11 which is moving in the direction of the arrow of Fig. 1. In Fig. 4 the conveyor belt is moving parallel to the direction of pulp web 8.

5 The conveyor belt 11 moves at successively increasing and decreasing speeds by means of any suitable mechanism, such as a cam. Because of the successively increasing and decreasing speeds the pulp webs are piled up 10 in successively decreasing and increasing quantities as illustrated in Figs. 3, 5 and 6, the exposed fold edges being spaced at increasing and decreasing distances. By properly regulating the maximum and minimum 15 speeds of conveyor 11 the degree of taper between points of minimum and maximum thickness may be varied at will.

The pulp web, when laid down transversely to the conveyor 11 of Figs. 1 and 2, forms 20 a series of overlapping folds of pulp illustrated in Fig. 3, the distances between the edges varying with the speed of the conveyor, that is, increasing and decreasing regularly 25 according to the increasing and decreasing speed of the conveyor 11. The folds may be cut at the folded edges as shown by the arrows in Fig. 7 or may be used in the form shown. The folded edges come at the edge 30 of the fibrous sheet but are not parallel to it and must be trimmed. It is necessary to proportion the width of the pulp web to the length of the taper and the speed of the conveyor 11. The fibers when laid down 35 transversely are at an angle greater than 45° to the machine direction of conveyor 11, and are substantially at right angles to it. A fibrous sheet or board made in this manner has greater strength across the sheet than 40 with the machine direction.

If the folds of pulp web are laid down 45 parallel to the machine direction by the machine of Fig. 4, the folded edges are across the sheet as shown in Fig. 5. The folds of pulp web made by this method extend from one surface of the fibrous sheet diagonally through to the other surface.

The fibrous sheet or board formed by laying down the folds of pulp web parallel or 50 transversely to the direction of the conveyor 11, or in any other predetermined manner as may seem desirable, usually passes through a continuous press 13, which may be in the form of press-rolls. This operation compresses the loosely piled overlapping folds 55 of pulp web into a homogeneous and coherent moist fibrous sheet or board. If the paper has been creped by doctor 6, the pressure of rolls or other press 13 interlocks the creped 60 paper surfaces to form a fibrous sheet in which the overlapping folds adhere at their surfaces with greater tenacity than when the moist webs are not creped. The moist fibrous sheet may either be dried or used as a moist 65 pulp product without drying after leaving

the continuous press 13. If the product is to be dried the sheet then passes through drier 14, after which it may pass through trimmer 15 and cutter 16.

A board made in the manner outlined 70 above presents a longitudinal contour which is rounded at the points of maximum and minimum thickness, as illustrated in an exaggerated manner in Fig. 8. For shingles it is desirable that the tapered surface proceed 75 in a uniform plane from the line of maximum thickness to that of minimum thickness and that there be an angular break in the longitudinal contour line at the points where the direction of taper changes. Plane surfaces 80 and angularity may be obtained by introducing a shaping operation into the process of manufacture.

The drier 14 may be regulated so as not to completely dry the sheet. The cutter 16 85 may cut the continuous sheet at lines of minimum thickness only. The cutter 16 may be followed by a conveyor traveling at right angles to the previous direction of travel. This latter conveyor may carry the tapered 90 double sheets through heated press rolls 21 and 22, as shown in Fig. 10. The upper rolls 21 are inclined at an angle conforming with the taper of the sheet and have uniform downward pressure acting upon their bearings. 95 These press rolls exert a shaping action upon the sheet in addition to a pressing and drying action. The tendency of the contour of the sheet to become rounded at points of maximum and minimum thickness is thus 100 corrected and a product is secured which possesses the desired plane surfaces and sharp angles.

For practical purposes, preliminary drier 17', as shown in Fig. 11, may be interposed 105 between felt 4 and conveyor 7 of the machine shown in Figs. 1, 2 and 4. The moist pulp web winds over a plurality of rolls 18. During the passage through drier 17' the web is maintained in contact with a stream of warm 110 dry air which enters at inlet pipe 19 and exhausts at the outlet pipe 20. The drier is arranged to remove a portion, approximately 20%, of the moisture contained in the web. Precautions must be observed not to remove 115 too much moisture since that will reduce the coherence of the resulting sheet. The preliminary drier is employed because moisture can be removed more efficiently from a single 120 web than from a thick sheet.

If the sheet is to be made of water-resisting as in the production of asphalt shingles, the finely divided water-resistant material may be suspended in the slurry of water and pulp 125 in vat 1 of the wet machine. The perforate cylinder mould 2 will then pick up a web of pulp and water-resistant material. The pulp web 8 will contain the water-resistant material, such as asphalt, and the built up board will have it disseminated throughout. In an 130

other method, as described in the Weiss application, the water-resistant compound may be dusted or sprayed in finely divided form on the pulp web 8. A suitable device for this purpose is illustrated diagrammatically at 5 8' in Fig. 2 of the drawings. In such a method, better adherence between the water-resistant compound and the wet web is secured if a small amount of water-resistant compound has been previously incorporated 10 in the slurry in vat 1. The overlapping pulp folds containing the water-resistant compound such as asphalt are then passed through heated press rolls to dry the pulp and melt the water-resistant compound and thereby thoroughly saturate the fibrous sheet or board. The board may be given a further 15 coating of water-resistant compound followed by a layer of crushed rock to complete the shingle surface.

Throughout the claims the term "folds" is used to define, not only the folded edge, but the entire overlapping portions formed by each reciprocation of the looping device, and 20 the term "edge" when used in conjunction with "folds" is intended to mean either the folded edge or loop, or the non-folded side edge of the portion of the web forming the folds.

30 Various other changes may be made in the fibrous sheets and in the methods of fabricating these sheets without departing from the spirit of the invention as defined by the appended claims.

35 I claim:

1. As an article of manufacture a fibrous sheet successively increasing and decreasing in thickness along the machine direction of said sheet, comprising overlapping folds of 40 pulp web having edges extending in transverse relation to the machine direction of said sheet, said edges being spaced from each other in the machine direction of the finished sheet in successive series of decreasing and increasing distances.

45 2. As an article of manufacture a fibrous sheet successively increasing and decreasing in thickness along the machine direction of said sheet, comprising overlapping creped folds of pulp web having edges extending in transverse relation to the machine direction of said sheet, said edges being spaced from each other in the machine direction of the finished sheet in successive series of decreasing and increasing distances.

50 3. As an article of manufacture, a paper board successively increasing and decreasing in thickness along the machine direction of said board, comprising a pressed sheet of overlapping folds of paper-stock web having edges extending in transverse relation to the machine direction of said board, said edges being spaced from each other in the machine direction of the finished board in successive 55 series of decreasing and increasing distances.

4. As an article of manufacture, a paper board successively increasing and decreasing in thickness along the machine direction of said board, comprising a pressed sheet of overlapping folds formed from a single web 70 of paper-stock having edges extending in transverse relation to the machine direction of said board, said edges being spaced from each other in the machine direction of the finished board in successive series of decreasing and increasing distances.

5. As an article of manufacture, a paper board successively increasing and decreasing in thickness along the machine direction of said board, comprising a pressed sheet of overlapping folds of paper-stock web having edges extending in transverse relation to the machine direction of said board, said edges being spaced from each other in the machine direction of the finished board in successive 80 series of decreasing and increasing distances, the majority of the fibers of said board being at an angle greater than 45° to the machine direction of said board.

6. As an article of manufacture, a coherent paper board successively increasing and decreasing in thickness along the machine direction of said board, comprising a pressed sheet of overlapping folds of pulp web having edges extending in transverse relation to the machine direction of the sheet, said edges being spaced from each other in the machine direction of the finished board in successive series of decreasing and increasing distances and having the constituent folds at an angle 90 to the finished surfaces.

7. As an article of manufacture a fibrous sheet successively increasing and decreasing in thickness along the machine direction of said sheet and having the constituent 105 fibrous webs at an angle to the finished surfaces.

8. As an article of manufacture a water-resistant fibrous sheet successively increasing and decreasing in thickness along the machine direction of said sheet and having the constituent fibrous webs at an angle to the finished surfaces.

9. As an article of manufacture an asphalt saturated fibrous sheet successively increasing and decreasing in thickness along the machine direction of said sheet and having the constituent fibrous webs at an angle to the finished surfaces.

10. As an article of manufacture a fibrous sheet successively increasing and decreasing in thickness along the machine direction of said sheet.

11. As an article of manufacture a coherent paper board successively increasing and decreasing in thickness along the machine direction of said board.

12. The method of making a fibrous sheet successively increasing and decreasing in thickness which comprises laying down over-

lapping folds of moist pulp webs on a conveyor moving at successively decreasing and increasing speeds and then pressing said moist pulp webs into a coherent sheet.

13. The step in the method of making a fibrous sheet successively increasing and decreasing in thickness which comprises laying down overlapping folds of moist pulp webs on a conveyor moving at successively decreasing and increasing speeds.

14. The method of making a fibrous sheet successively increasing and decreasing in thickness which comprises laying down a moist pulp web continuously and transversely on a conveyor moving at successively decreasing and increasing speeds to form overlapping folds, and pressing said pulp webs into a coherent sheet.

15. The method of making a fibrous sheet successively increasing and decreasing in thickness which comprises partially drying a moist pulp web, laying down said partially dried web upon a conveyor moving at successively decreasing and increasing speeds to form overlapping folds, and pressing said overlapping folds into a coherent sheet.

16. The method of making a fibrous sheet having uniformly tapered plane surfaces which comprises laying down a moist pulp web on a conveyor moving at successively decreasing and increasing speeds to form overlapping folds, pressing said pulp webs into a coherent sheet, and heating and pressing said sheet to remove the moisture therefrom and to form plane tapered surfaces thereon.

17. The steps in the method of making tapered shingles which comprise laying down a moist pulp web continuously on a conveyor moving at successively decreasing and increasing speeds to form overlapping folds, pressing said pulp webs into a coherent sheet, and cutting said pressed sheet into short lengths along the lines of maximum and minimum thickness.

18. The method of making water-resistant, tapered shingles which comprises forming a suspension of pulp and finely divided water-resistant material, forming a continuous moist web from said pulp and water-resistant material, laying down said moist web continuously on a conveyor moving at successively decreasing and increasing speeds to form overlapping folds, pressing and heating said overlapping webs to dry, bind and saturate said webs with said water-resistant material and form a coherent sheet, and cutting said pressed sheet into short lengths along the lines of maximum and minimum thickness.

19. The method of making water-resistant tapered shingles which comprises forming a suspension of pulp and finely divided water-resistant material, forming a continuous moist web from said pulp and water-resist-

ant material, spraying said moist web with an additional quantity of water-resistant material, laying down said moist web continuously on a conveyor moving at successively decreasing and increasing speeds to form overlapping folds, pressing and heating said overlapping webs to dry, bind and saturate said webs with said water-resistant material and form a coherent sheet, and cutting said pressed sheet into short lengths along the lines of maximum and minimum thickness.

20. The method of making tapered shingles which comprises forming a suspension of pulp and finely divided water-resistant material, forming a moist web from said pulp, partially drying said moist web, laying down said partially dried web continuously on a conveyor moving at successively decreasing and increasing speeds to form overlapping folds, pressing said overlapping, partially dried folds to form a coherent sheet, drying said pressed sheet, and cutting said dried sheet into short lengths along lines of maximum and minimum thickness.

21. The steps in the method of making a uniformly tapered shingle which comprise laying down a moist pulp web continuously on a conveyor moving at successively decreasing and increasing speeds to form overlapping folds, pressing said pulp webs into a coherent sheet, cutting said pressed sheet into individual lengths along the lines of minimum thickness, pressing and heating said individual lengths to dry said lengths and to form plane tapered surfaces thereon, and cutting said individual lengths along the lines of maximum thickness.

22. In a machine for making a fibrous tapered sheet the combination of means for forming overlapping folds of pulp webs and means for spacing said folds in the machine direction of the finished sheet in a series of regularly increasing and decreasing distances.

23. In a machine for making a fibrous tapered sheet, the combination of means for laying down a moist pulp web in overlapping folds, means for spacing said folds in the machine direction of the finished sheet in a series of regularly increasing and decreasing distances, and means for pressing said succession of folds into a coherent sheet.

24. In a machine for making a fibrous tapered sheet, the combination of means for creping a moist pulp web, means for laying down said creped web in overlapping folds, means for spacing said folds in the machine direction of the finished sheet in a series of regularly increasing and decreasing distances, and means for pressing said folds into a coherent sheet.

25. In a machine for making a fibrous tapered sheet, the combination of means for partially drying a moist pulp web, means for lay-

ing down said partially dried web in overlapping folds, means for spacing said folds in the machine direction of the finished sheet in a series of regularly increasing and decreasing distances, and means for pressing said folds into a coherent sheet.

26. A machine for making a fibrous tapered sheet, comprising means for forming a moist pulp web, means for partially drying said moist web, means for laying down said partially dried web in overlapping folds, means for spacing said folds in the machine direction of the finished sheet in a series of regularly increasing and decreasing distances, 10 means for pressing said folds into a coherent sheet, and means for drying said sheet.

27. A machine for making fibrous, water-resistant tapered shingles which includes the combination of means for forming moist webs 20 of pulp and finely divided water-resistant material, means for partially drying said moist webs, means for spraying additional water-resistant material upon said partially dried webs, means for laying down said treated webs in overlapping folds, means for spacing said folds in the machine direction of the resulting sheet in a series of regularly increasing and decreasing distances, means for pressing said folds into a coherent sheet, 25 means for drying said sheet, and means for cutting said dried sheet along the lines of maximum and minimum thickness.

28. In a machine for making a fibrous tapered sheet, a conveyor adapted to be driven 35 at varying speeds, and means for laying down a moist pulp web on said conveyor in overlapping folds.

29. In a machine for making a fibrous tapered sheet, a conveyor adapted to be driven 40 at varying speeds, and a reciprocating feeding device adapted to deliver a moist pulp web to said conveyor in overlapping folds.

In testimony whereof I affix my signature.  
**MAX KLIEFOTH.**